

## UNITED STATES PATENT OFFICE

HEINRICH FINK AND PAUL ESELLEMAN, OF PREMNITZ, WESTHAVELAND, GERMANY,  
ASSIGNORS TO I. G. FARBNINDUSTRIE AKTIENGESELLSCHAFT, OF FRANKFORT-  
ON-THE-MAIN, GERMANY, A CORPORATION OF GERMANY

## MANUFACTURE OF ARTIFICIAL FIBERS

No Drawing. Application filed March 6, 1929, Serial No. 344,910, and in Germany March 14, 1928.

Our present invention relates to a new process for manufacturing products of viscose in the form of threads, bands, etc. One of its objects relates to a new coagulating liquid. Another object of our invention is to provide fine viscose silk, spun from unmatured viscose obtained from unmatured or matured alkali cellulose, with a high wet and dry tensile strength. Additional objects of our invention are the new threads. Further objects of our invention will be seen from the detailed specification following hereafter.

Our invention is based on the observations that viscose, when brought into the form of threads, bands, etc., is coagulated by an acid ester, made by partly esterifying a polybasic mineral acid with an alcohol, the alkyl groups of which may be substituted. The products thus obtainable have excellent properties especially a high wet and dry tensile strength. As a precipitating liquid we may use, for instance, a mono ester of sulfuric acid or a mono or di-ester of phosphoric acid. These acids may be partly esterified with a monovalent aliphatic alcohol, such as methyl alcohol, ethyl alcohol, propyl alcohol or with an araliphatic alcohol, such as benzyl alcohol, or with a polyvalent alcohol, such as glycol, glycerin, trimethylene glycol or with a substituted alcohol, such as glycolic acid. Other substituted alcohols forming acid esters with polybasic mineral acids may be used in the same manner.

The action of our new precipitating liquids may be explained as follows:

A dibasic acid, for instance, sulfuric acid, becomes monobasic by esterification of one of its hydroxyl groups with an alcohol and thus forms a precipitating agent which shows, even in undiluted form, only half the acidity of sulfuric acid. Therefore, the partly esterified compound can be applied in a concentration much higher than the mineral acid itself without damaging the regenerated cellulose fiber.

This may be proved, for instance, by the following test:—

When treating a finished artificial fiber having a titer of 1 denier with sulfuric acid

of about 75% strength, the fiber is damaged in 20 to 30 seconds. Even by a sulfuric acid of 60% strength the filament is damaged in about 2 minutes. In contradistinction thereto, when using monomethyl sulfuric acid (prepared in the usual manner from two parts of concentrated sulfuric acid and one part of methyl alcohol), the fiber remains unaltered for 3-4 hours.

It is not necessary to use the partly esterified acid in a chemically pure form when carrying out our process on a large scale. A suitable precipitating bath is obtainable, for instance, by mixing equimolecular parts of the alcohol with the concentrated polybasic mineral acid or with its anhydride or with the corresponding acid chloride, care being taken that the temperature of the mixture is regulated in such a manner that the best possible yield of the ester is obtained.

In our precipitating bath an excess of the acid or the alcohol may be employed. As a rule, when using an excess of the acid, a more rapidly acting precipitating bath is formed, while an excess of alcohol diminishes the coagulating action. A coagulating bath thus obtained may be diluted with water within certain limits. This will be much more important when acid esters of high molecular weight or polyvalent alcohols are employed, these acid esters having a not desired high viscosity in undiluted state. In such cases, when the esters are not easily saponified in the presence of water up to 30% water may be added to the precipitating bath. In any case, however, the precipitating liquid shall contain at least 30% of the acid esters in question. Inorganic salts which are soluble in our precipitating bath may be added, for instance, sodium sulfate, sodium bisulfate, ammonium sulfate, zinc sulfate, sodium bisulfite.

Our new precipitating baths are especially useful in the manufacture of fine artificial threads of 3-1 deniers and even of finer fibers from an unmatured viscose prepared from unmatured alkali cellulose, for instance, according to U. S. Patent 1,428,246. Good results may even be obtained by subjecting the alkali cellulose to a previous ripening process

whereas the viscose is not allowed to mature. When using our new precipitating bath without special stretching apparatus, an artificial silk is obtainable which has a high luster, a very soft feel and a dry tensile strength of about 2 grams or more per denier and a wet tensile strength of about 1.3 grams per denier. These excellent properties may even be improved by stretching the thread in the course of its manufacture. To increase the luster and the soft feel of the threads, there may be added to the precipitating bath, for instance, a condensation product of a naphthalene sulfonic acid with formaldehyde, a sulfonated phenol resin, purified sulfite cellulose waste liquor, a carbazol sulfonic acid, a sulfonated cumaron resin, a sulfonated lubricating oil, a sulfonated brown coal tar oil, a tetrahydronaphthalene sulfonic acid, etc. If desired, the same or similar products may be already added to the viscose itself.

The threads may be stretched in any known manner while in the precipitating bath or after they have been removed from it, that is, between the spinning bath and the collecting device, such as a bobbin or centrifuge. This may be done, for example, by choosing a longer way between the bath and the collecting device or by leading the threads over rods or rolls arranged in such a manner in the bath or between the bath and the collecting device that the threads form one or more angles on their way, or by using a suitable thread guide or by leading them into a second bath in which they may be simultaneously freed from the adhering coagulating liquid.

The length of the thread immersed in the spinning bath may be varied within wide limits, for example, from 5 to 100 centimeters, said limits depending generally upon the temperature and nature of the coagulating bath and of the nature of the viscose solution applied. We prefer to keep the spinning bath at ordinary temperature, it may, however, likewise be varied within wide limits, and good results are obtainable at temperatures of about 0° to 40° C. The drawing speed of spinning may be varied up to 75 meters per minute, depending partly upon the temperature and nature of the bath, partly upon the length of immersion and the thickness of the thread, partly upon the viscosity of the spinning solution and finally upon the quantity of viscose solution pressed into the precipitating bath.

The following examples serve to illustrate the invention without limiting it thereto:

*Example 1.*—100 kilograms of methyl alcohol of 99% strength are mixed with 200 kilograms of sulfuric acid of 96% strength, the temperature of the mixture being kept for 2 hours at 40–50° C. By this time the acidity of the mixture has become stable as proved by titration. From the difference between the total amount of 64–66% by weight of sul-

furic acid and the total acidity of the mixture of about 41% of acid (calculated as H<sub>2</sub>SO<sub>4</sub>) it is found that the bath contains about 18% by weight of sulfuric acid monohydrate and about 52–53% of mono-methyl-ester of sulfuric acid, the remainder being unaltered methyl alcohol and water formed by the esterification. 70

A viscose solution containing 5–6% of cellulose and 5–7% of NaOH prepared from an entirely unmatured alkali cellulose, for instance, according to U. S. Patent 1,428,246 is pressed immediately after dissolving and filtering into a precipitating bath prepared as described above. Through a spinning opening of about 0.1 millimeter diameter at a drawing speed of about 30 meters per minute the viscose pump delivers such a quantity of viscose that a thread of 1 denier is formed. The temperature of the bath is kept at about 15–20° C., the length of immersion being about 50–100 centimeters. After having passed the precipitating bath, the thread is guided over rods or rolls into a second bath where it is washed with water and then to a collecting device, for instance, to a bobbin, irrigated with fresh water. The well washed threads are freed from sulfur, bleached and finished in the usual manner known in the viscose art. 95

*Example 2.*—The same viscose solution as mentioned in Example 1 is spun under the same conditions into the same bath but at a bath temperature of 35° C. and a length of immersion of 15 centimeters. 100

*Example 3.*—The same viscose as described in Example 1 is spun with a length of immersion of 30 centimeters into a coagulating bath, made by mixing of 100 kilograms of ethyl alcohol of 95% strength with 200 kilograms of concentrated sulfuric acid of 96% strength and heating until the esterification has been finished. The precipitating bath contains about 49% of ethyl sulfuric acid and 27% of sulfuric acid. By glass rods of suitable thickness there are imparted so much angles to the filament that spinning is still possible. All the other conditions are the same as described in Example 1. 110

*Example 4.*—The same viscose as described in Example 1, is spun under the same conditions as in Example 3 but with a length of immersion of 40 centimeters into a precipitating bath, made of 200 kilograms of technical butyl alcohol and 400 kilograms of concentrated sulfuric acid. In order to diminish the high viscosity of the finished reaction mixture 100 kilograms of water are added. The bath contains about 53% of butyl sulfuric acid and 23% of sulfuric acid. 115 120 125

*Example 5.*—The same viscose as described in Example 1, is spun with a length of immersion of 15 centimeters into a precipitating bath kept at a temperature of 15–20° C. which is made in the following way:— 130

100 kilograms of methyl alcohol of 99% strength are mixed with 300 kilograms of sulfuric acid of 96% strength and stirred, the temperature being kept at 50° C. for 2 hours. 5 The acidity determined by titration and calculated as  $H_2SO_4$ , amounts to 49.2%. Hence follows a content 52.5% of methyl sulfuric acid and 26% of sulfuric acid in the bath. The other conditions are the same as in Example 1.

10 *Example 6.*—The same viscose as described in Example 1, is pressed into a bath made by introducing 70 kilograms of phosphoric acid anhydride into 50 kilograms of methyl alcohol. The mixture, after filtering from the undissolved, titrated with baryta water, contains 46.3% of monomethyl phosphoric acid 34.9% of dimethyl phosphoric acid and 3.2% of phosphoric acid. Before using it 30% of 20 water is added to the bath. The length of immersion amounts to 20 centimeters, the bath temperature is 15° C. The drawing speed amounts to about thirty five meters per minute. The viscose pump delivers such a 25 quantity of viscose that a thread of 1 denier is formed.

15 *Example 7.*—The same viscose and acid as described in Example 5 are used. The viscose pump however is caused to deliver the double 30 quantity of viscose so that a thread of 2 denier is formed. The diameter of the spinning openings amounts to 0.08 millimeters.

20 *Example 8.*—The same viscose and acid as described in Example 5 are used. But the 35 viscose pump is caused to deliver such a quantity of viscose, that a thread of 0.5 denier is formed. The diameter of the spinning openings amounts to 0.08 millimeters.

25 *Example 9.*—The same viscose as described 40 in Example 1, is spun through a nozzle having 600 spinning openings of 0.1 millimeter diameter at a drawing speed of about sixty meters per minute into a precipitating bath of a length of 60 centimeters of the same composition as described in Example 1, at a temperature of 25° C. while stretching over several glass rods upon a reel which is irrigated with water. The hank is cut off, washed, finished and prepared for staple fibers.

30 *Example 10.*—An alkali cellulose, made by immersing one part of sulfite cellulose in 15 parts of caustic soda solution containing 18% of its weight of NaOH at the temperature of 13° C. for two hours after having been 35 pressed to the triple weight of cellulose and disintegrated, is matured four days at a temperature of 18° C. The matured alkali cellulose is well xanthogenized with a quantity of carbon disulfide amounting to 40-50% of 40 the weight of cellulose, the formed xanthogenate being thereafter dissolved at a temperature below +10° C. to a viscose containing 7-8% of cellulose and 6-7% of NaOH. The finished viscose, which does not show any 45 ammonium chloride titer according to Hot-

tenroth is spun immediately according to the arrangement and with the acid described in Example 1. The quantity of viscose to be delivered from the pump and the speed of drawing must be adapted in a manner as to 50 form a thread of 1 denier.

75 *Example 11.*—From the same alkali cellulose as described in Example 10, a viscose is made containing 7-8% of NaOH and 10% of cellulose with the same viscosity. It is spun as described in Example 10 into the same precipitating bath, the quantity of viscose to be delivered from the pump being 3.2 ccm per minute. A drawing speed of about 30 centimeters per minute is maintained so that, when applying a spinning nozzle of 120 spinning openings with a diameter of 0.08 millimeters, 80 a thread with the titer of 1 denier is obtained.

85 The threads thus obtainable have a dry tensile strength of 3 grams and more per denier and in the wet state 1.8 to 3 grams per denier. Dry and wet stretching amounts to 5-8%. They have an excellent soft feel and luster; the luster is a little duller than that 90 of the usual artificial silks; their capacity of being dyed equals to that of other viscose silk prepared in the usual manner. Owing to their high tensile strength, they are well fit for being worked on textile machines.

95 In the following claims the expression "an acid ester of polybasic mineral acid with an aliphatic alcohol" is intended to include all products which are obtainable by partly esterifying a polybasic mineral acid with an aliphatic alcohol which may be substituted:—When using the expression "completely 100 unmatured viscose," we mean unmatured viscose prepared from an unmatured alkali cellulose, for instance, in accordance with U. S. Patent 1,428,246.

105 Having now particularly described and ascertained the nature of our said invention and in what manner the same is to be performed, we declare that what we claim is:

110 1. The process for manufacturing artificial fibers from viscose, which comprises pressing a viscose solution through a spinning nozzle into a precipitating bath containing at least 30% of an acid ester of a polybasic mineral acid with an aliphatic alcohol. 115

2. The process for manufacturing artificial fibers from viscose, which comprises pressing a viscose solution through a spinning nozzle into a precipitating bath containing at least 30% of an acid ester of a polybasic mineral acid with a monovalent aliphatic alcohol. 120

3. The process for manufacturing artificial fibers from viscose, which comprises pressing a viscose solution through a spinning nozzle into a precipitating bath containing at least 30% of a methyl ester of a polybasic mineral acid. 125

4. The process for manufacturing artificial fibers from viscose, which comprises pressing a viscose solution through a spin- 130

ning nozzle into a precipitating bath containing at least 30% of an acid ester of sulfuric acid with an aliphatic alcohol.

5. The process for manufacturing artificial fibers from viscose, which comprises pressing a viscose solution through a spinning nozzle into a precipitating bath containing at least 30% of an acid ester of sulfuric acid with a monovalent aliphatic alcohol.

10. 6. The process for manufacturing artificial fibers from viscose, which comprises pressing a viscose solution through a spinning nozzle into a precipitating bath containing at least 30% of sulfuric acid monomethyl ester.

15. 7. The process for manufacturing artificial fibers from viscose, which comprises pressing a viscose solution through a spinning nozzle into a precipitating bath obtained by esterifying about molecular proportions of sulfuric acid and of a monovalent aliphatic alcohol.

20. 8. The process for manufacturing artificial fibers from viscose, which comprises pressing a viscose solution through a spinning nozzle into a precipitating bath obtained by esterifying about molecular proportions of sulfuric acid and of methyl alcohol.

25. 9. The process for manufacturing artificial fibers from viscose, which comprises pressing a viscose solution through a spinning nozzle into a precipitating bath containing at least 30% of an acid ester of a polybasic mineral acid with an aliphatic alcohol and stretching the freshly coagulated threads.

30. 10. The process for manufacturing artificial fibers from viscose, which comprises pressing a viscose solution through a spinning nozzle into a precipitating bath containing at least 30% of an acid ester of a polybasic mineral acid with a monovalent aliphatic alcohol and stretching the freshly coagulated threads.

35. 11. The process for manufacturing artificial fibers from viscose, which comprises pressing a viscose solution through a spinning nozzle into a precipitating bath containing at least 30% of a methyl ester of a polybasic mineral acid, and stretching the freshly coagulated threads.

40. 12. The process for manufacturing artificial fibers from viscose, which comprises pressing a viscose solution through a spinning nozzle into a precipitating bath containing at least 30% of an acid ester of sulfuric acid with an aliphatic alcohol, and stretching the freshly coagulated threads.

45. 13. The process for manufacturing artificial fibers from viscose, which comprises pressing a viscose solution through a spinning nozzle into a precipitating bath containing at least 30% of an acid ester of sulfuric acid

with a monovalent aliphatic alcohol, and stretching the freshly coagulated threads.

14. The process for manufacturing artificial fibers from viscose, which comprises pressing a viscose solution through a spinning nozzle into a precipitating bath containing at least 30% of sulfuric acid monomethyl ester, and stretching the freshly coagulated threads.

15. The process for manufacturing artificial fibers from viscose, which comprises pressing a viscose solution through a spinning nozzle into a precipitating bath obtained by esterifying about molecular proportions of sulfuric acid and of a monovalent aliphatic alcohol, and stretching the freshly coagulated threads.

16. The process for manufacturing artificial fibers from viscose, which comprises pressing a viscose solution through a spinning nozzle into a precipitating bath obtained by esterifying about molecular proportions of sulfuric acid and of methyl alcohol, and stretching the freshly coagulated threads.

17. The process for manufacturing artificial fibers from viscose, which comprises pressing a viscose solution through a spinning nozzle into a precipitating bath containing at least 30% of an acid ester of a polybasic mineral acid with an aliphatic alcohol and immediately subjecting the freshly formed threads to a washing operation.

18. The process for manufacturing artificial fibers from viscose, which comprises pressing a viscose solution through a spinning nozzle into a precipitating bath containing at least 30% of an acid ester of a polybasic mineral acid with a monovalent aliphatic alcohol and immediately subjecting the freshly formed threads to a washing operation.

19. The process for manufacturing artificial fibers from viscose, which comprises pressing a viscose solution through a spinning nozzle into a precipitating bath containing at least 30% of a methyl ester of a polybasic mineral acid and immediately subjecting the freshly formed threads to a washing operation.

20. The process for manufacturing artificial fibers from viscose, which comprises pressing a viscose solution through a spinning nozzle into a precipitating bath containing at least 30% of an acid ester of sulfuric acid with an aliphatic alcohol and immediately subjecting the freshly formed threads to a washing operation.

21. The process for manufacturing artificial fibers from viscose, which comprises pressing a viscose solution through a spinning nozzle into a precipitating bath containing at least 30% of an acid ester of sulfuric acid with a monovalent aliphatic alcohol and immediately subjecting the freshly formed threads to a washing operation.

22. The process for manufacturing arti-

5 ficial fibers from viscose, which comprises pressing a viscose solution through a spinning nozzle into a precipitating bath containing at least 30% of sulfuric acid monomethyl ester and immediately subjecting the freshly formed threads to a washing operation.

10 23. The process for manufacturing artificial fibers from viscose, which comprises pressing a viscose solution through a spinning nozzle into a precipitating bath obtained by esterifying about molecular proportions of sulfuric acid and of a monovalent alcohol and immediately subjecting the freshly 15 formed threads to a washing operation.

15 24. The process for manufacturing artificial fibers from viscose, which comprises pressing a viscose solution through a spinning nozzle into a precipitating bath obtained by esterifying about molecular proportions of sulfuric acid and of methyl alcohol and immediately subjecting the freshly 20 formed threads to a washing operation and stretching the coagulated threads.

25 25. A precipitating bath for manufacturing artificial fibers from viscose containing at least 30% of an acid ester of sulfuric acid with a monovalent aliphatic alcohol.

30 26. A precipitating bath for manufacturing artificial fibers from viscose containing at least 30% of an acid ester of sulfuric acid with a monovalent aliphatic alcohol to which ester up to 30 per cent. of water is added.

35 27. A precipitating bath for manufacturing artificial fibers from viscose containing at least 30% of sulfuric acid monomethyl ester.

40 28. The process for manufacturing artificial fibers from viscose, which comprises pressing an unmatured viscose into a precipitating bath containing at least 30% of an acid ester of sulfuric acid with a monovalent aliphatic alcohol.

45 29. The process for manufacturing artificial fibers from viscose, which comprises pressing an unmatured viscose into a precipitating bath containing at least 30% of sulfuric acid monomethyl ester.

50 30. The process for manufacturing artificial fibers from viscose, which comprises pressing a completely unmatured viscose into a precipitating bath containing at least 30% of an acid ester of sulfuric acid with a monovalent aliphatic alcohol.

55 31. The process for manufacturing artificial fibers from viscose, which comprises pressing a completely unmatured viscose into a precipitating bath containing at least 30% of sulfuric acid monomethyl ester.

60 32. Artificial fibers consisting of regenerated cellulose having a dry tensile strength of more than 2 grams per denier and a wet tensile strength of more than 1.25 grams per denier, obtained by the process as claimed in 65 claim 1.

33. Artificial fibers consisting of regenerated cellulose having a dry tensile strength of more than 3 grams per denier and a wet tensile strength of 2 grams and more per denier, obtained by the process as claimed in 70 claim 9.

34. The process for manufacturing artificial fibers from viscose which comprises pressing a viscose solution through a spinning nozzle in a precipitating bath containing at least 30% of sulfuric acid monomethyl ester and about 18% of sulfuric acid monohydrate. 75

35. A precipitating bath for manufacturing artificial fibers from viscose containing at least 30% of sulfuric acid monomethyl ester and about 18% of sulfuric acid monohydrate. 80

In testimony whereof, we affix our signatures.

85 HEINRICH FINK.  
PAUL ESSELMANN.

90

95

100

105

110

115

120

125

130